

## UNITED STATES PATENT OFFICE

2,194,610

## PROCESS FOR MANUFACTURING WHITE LEATHER

August C. Orthmann, Milwaukee, Wis., and Fred C. Wright, Glen Ellyn, Ill., assignors to R. T. Vanderbilt Co. Inc., New York, N. Y., a corporation of New York

No Drawing. Application March 19, 1937,  
Serial No. 131,882

6 Claims. (Cl. 149—7)

This invention relates generally to the manufacture of leather and more particularly to a process for incorporating pigments in hides, skins, or the like during the tanning thereof.

5 The invention, while applicable with especial advantages to the manufacture of white leather by the chrome tanning process, may also be used for incorporating various other pigments in hides or skins. For example, not only whites but various shades of chrome yellows, chrome greens, blues and reds (iron oxides) may be used. And the process of the present invention may also be employed in connection with the vegetable tanning of sheep skin, calf skin, and the like, when 10 the tanning operation is effected by milling the skins in drums in the presence of a suitable tanning liquor.

For the sake of illustration or example the invention will be described in detail as applied to 20 the manufacture of white leather by the chrome tanning process.

Heretofore in the manufacture of leather of this character the white pigments employed have been applied to the leather while it is being fat 25 liquored or just before the fat liquoring operation. At such time the leather is tightened up, that is, is relatively impervious or non-porous and, as a consequence, the added pigment has had only a surface effect on the grain side of the 30 leather, the underlying body of the leather or intermediate portion of the hide remaining dark in color. As a result, there is a marked or substantial contrast between the whitened surface of the leather and the dark colored body underlying such surface. The hiding power of the 35 pigment is overtaxed and the desired color effect is lacking. A true white leather is not obtained. And, in many instances, the whitened surface being constituted differently from the underlying body of the leather is in an unstable condition with the consequence that the color or appearance of its surface may be impaired after the leather has been in use for a short time.

One of the objects of the present invention is 40 to secure a complete and effective impregnation or penetration of the pigment throughout not only the surface but also the body of the leather and to accomplish this in such a way that the quality of the leather is not, in any way, impaired. While the concentration of the pigment 45 may be somewhat greater in the region of the surface at the grain side of the leather than in the interior of the body thereof, there is a complete and substantially uniform impregnation so that the interior is toned down to approximate

the color of the surface of the grain side and the resulting leather is substantially or practically homogenous in its pigment content. This eliminates any sharp or decided contrast between the color of the body of the leather and the surface thereof thereby making full use of the hiding power of the pigment and bringing about a stable condition so that the leather will retain its color or appearance even when rubbed or subjected to an abrading action.

Generally speaking, these desirable results are obtained by milling the pigment into the leather in rotating drums while the leather is in an open, porous condition and when the open fibers of the leather are pervious to rather complete penetration by the pigment. This may be advantageously accomplished in the early stages of either chrome or vegetable tanning and with various pigments.

In chrome tanning, after the hides, skins, or the like are unhaired, they are bated and pickled and then chrome tanned, that is, the hides are milled in suitable drums in a suitable liquor or solution containing a basic chromium salt.

At this time the hides are, as indicated, in an open porous, fibrous condition. The present invention proposes to incorporate the pigment in the leather during the chrome tanning and for this purpose the pigments are added to the chrome tanning liquor at the beginning of the chrome tanning operation, and are worked into the leather while the hides are being milled in the rotating drums in the presence of the chrome tanning liquor. One pigment which may be advantageously employed is an oxide of titanium or a mixture of titanium dioxide and lithopone. Where such a mixture is employed one pound of titanium dioxide to four pounds of lithopone is employed, the proportions depending on the opacity of the lithopone. The amount of pigment employed is from five to fifteen per cent (by weight) to that of the pickled hides, although this may vary with the hides or skins to be treated. Other well-known pigments, for example antimony oxide, or the so-called extended pigments with titanium as a base may be used.

The hides are usually milled in the drums in the tanning liquor and pigment for from five to eight hours. The stock is then neutralized with an alkali to the proper degree after which it is mechanically handled, that is, taken out, piled up and drained. It is then wrung out and split and shaved, and next retanned in the same manner as before but in a shorter time. No pigment need be employed in the retanning operation.

If desired, it may then be bleached although the bleaching step may be omitted in many instances. Afterwards it is washed preparatory to being fat liquored. At this stage the hides are usually colored or fat liquored. In the present instance, the whitening of the hides may be toned by a suitable coloring or bleaching operation but of course the fat liquoring must be resorted to to lubricate the fibers and soften the leather.

10 The essential feature of the invention is the incorporation of the pigment in the hides while they are being milled in the drums during the early stages of the tanning operation and incidentally while they are in an open or porous fibrous condition. The other steps of the process may be varied. For example, the hides may be split and shaved after pickling instead of after the chrome tanning but where they are split and shaved after pickling they are then chrome tanned and pigmented as before.

Where the process is applied to vegetable tanning, the pigments are likewise worked into the skins or hides in an early stage of the tanning operation, that is, after the skins and hides have been unhaired, bated and pickled and when they are being milled in drums in the presence of a vegetable tanning liquor. The pigment is added to the tanning liquor as before and is milled into the hides or skins while they are in an open or porous, porous condition whereby thorough and complete penetration of the pigment throughout the skins or hides is realized.

In any event the pigment uniformly and completely penetrates the hides so that the interior thereof is whitened or so toned down as to blend in with and present no disadvantageous contrast to the whitened surface of the grain side of the leather. The hiding power of the pigment in the grain side thus operates to best advantage and since the pigmented leather is substantially homogenous or uniform as to pigment content and color, it is structurally stable as well as fast as to color. A quality leather of desired color and of durable character is had.

45 After the hides, skins, or the like have been processed and treated in the manner described, the leather may be finished in accordance with any standard or suitable practice.

From the foregoing it will be understood that 50 the present invention produces a new article of manufacture, namely, leather having not only the surface of its grain side but also its body impregnated with pigment, with the pigment content of the surface region and of the interior of the leather practically homogenous whereby 55 any undesirable contrast between the color of the surface and that of the interior is eliminated, the full hiding power of the surface pigment most advantageously utilized, and a surface of stable, durable structure is had.

60 While we have shown and described several ways in which the invention may be carried out, it is to be understood that the examples have been selected merely for the purpose of illustration and that various changes and substitution may be resorted to as will be understood by those skilled in the art without departing from the spirit of the invention or the scope of the subjoined claims.

The invention claimed is:

1. The herein-described process of manufacturing leather which comprises milling hides, skins, and the like in rotatable tanning drums in the presence of a tanning liquor and adding an insoluble pigment to the tanning liquor in the early 5 stages of the tanning operation and milling the pigment into the hides while they are in an open, porous condition.

2. The herein-described process of manufacturing leather which comprises milling the hides, 10 skins, and the like in rotatable drums and in the presence of a tanning liquor after they have been unhaired, bated and pickled and adding an insoluble pigment to the tanning liquor during the milling operation and milling the pigment into the 15 material while it is in an open, porous and porous condition to obtain a complete and practically uniform penetration of the pigment throughout the material.

3. The herein-described process of manufacturing leather which comprises unhauling, bathing and pickling the raw material, milling the raw material in a rotatable drum in the presence of tanning liquor containing a basic chromium salt, 25 and adding an insoluble pigment to the tanning liquor at the beginning of the milling of the raw material and milling the pigment into the material while it is in an open, porous and porous condition.

4. The herein-described process of manufacturing leather which comprises unhauling, bathing, and pickling the raw material, milling the raw material in a rotatable drum in the presence of tanning liquor containing a basic chromium salt, 35 and adding an insoluble white pigment containing an oxide of titanium to the tanning liquor during the milling of the material in the drum and milling the pigment into the material during the milling operation and causing it to uniformly penetrate the surface and body thereof. 40

5. The herein-described process of manufacturing leather which comprises unhauling, bathing and pickling the raw material, milling the raw material in a rotatable drum in the presence of tanning liquor containing a basic chromium salt, 45 and adding an insoluble pigment consisting of a mixture of titanium oxide and lithopone to the tanning liquor during the milling operation and milling the pigment into the material and causing it to uniformly impregnate the surface and body 50 thereof.

6. The herein-described process of manufacturing leather which comprises milling the hides, skins, and the like in rotatable drums and in the presence of a tanning liquor after they have been 55 unhaired, bated and pickled and adding an insoluble pigment to the tanning liquor during the milling operation and milling the pigment into the material while it is in an open, porous and porous condition to obtain a complete and practically uniform penetration of the pigment throughout the material, neutralizing and then mechanically handling the stock, split and shaving the same, retanning and then fat liquoring 60 the stock, and finishing the leather as desired. 65

AUGUST C. ORTHMANN.  
FRED C. WRIGHT.